

## UNITED STATES PATENT OFFICE

2,303,600

## DENTAL IMPRESSION MATERIAL

Constant A. Benoit and Herman C. Fuchs, Brooklyn, N. Y., assignors to Permatex Company, Inc., Brooklyn, N. Y., a corporation of New York

No Drawing. Application December 26, 1940,  
Serial No. 371,772

16 Claims. (Cl. 18—47)

As dental impression materials must necessarily be applied within the mouth and brought into intimate contact with its delicate tissues, they must possess specific properties and characteristics in order that they may successfully meet the peculiar conditions incident to their use.

From among the evident properties which should be possessed by a composition of matter adapted for the production of dental impressions, we mention the following: it should be ready for use or easily prepared for use as time is an important factor to the dentist; it should be of such physical condition that it can be readily inserted into the fissures and crevices of the soft and hard tissues of the mouth and readily removed therefrom without destruction of the impressions thereof; it should be of such chemical and physical condition as to allow of the production of accurate impressions without the use of heat; it should not require either heating or chilling in the mouth in order to accomplish its successful removal therefrom; it should be of such composition as to require a minimum of time for its application and removal; it should not break up, crumble, or separate in the mouth thus removing all possibility of its entering the throat; it should not generate heat through chemical reaction immediately before or during its application thus keeping the patient at ease and insuring a true impression under normal temperature conditions; it should be of such construction as to give sharp and accurate impressions; it should be of such composition as to be adapted for use in edentulous mouths as well as in those in which teeth are present; it should be of such composition that it will not cause the patient to gag; it should not expand or contract after the impression has been made; it should be readily removable from the model; it should not stick to the mouth surfaces; it should not be objectionable in taste or odor; it should be absolutely free from any deleterious or objectionable effect upon the mouth tissues; and it should be absolutely free from any poisonous or injurious materials.

The above-mentioned are only some of the characteristics which should be possessed by dental impression materials, but they are sufficient to indicate the care that must be taken in the preparation of such compositions and the

many requirements that must be met in the selection of the materials in their production.

Many attempts have been made to produce compositions of matter suitable for dental impressions but all of them, as far as we know, possess some of the above-mentioned objectionable features.

Among the objectionable components of previously described compositions suggested for use in the production of dental impressions is plaster of Paris, which generates heat during setting, is removed with difficulty; has a decided tendency to crack, flake, and break in the mouth and to drop into the throat of the patient; starts contracting a few hours after the impression has been made, and its use in general is objectionable to the patient.

Among other objectionable ingredients are those chemicals, such as gums and resins, requiring the use of objectionable solvents of an aromatic nature, turpentine, or methyl alcohol, all of which have an irritating effect upon the mouth tissues, and many of which are injurious if accidentally swallowed.

The hydro-colloids are particularly objectionable because of their susceptibility to expansion and contraction during their application for impressions and during the period between removal from mouth and preparation ("casting") of model, the resulting cast therefrom being different from the original mouth impression when such changes take place. The hydro-colloids are further objectionable because they are used warm. They must be chilled in the patient's mouth before an impression can be removed, which method requires the use of water-cooled impression trays. Furthermore, the hydro-colloids require long experience and very skillful manipulation before they can be used with a fair degree of confidence.

Waxes, which have been suggested for impression materials, also possess the highly objectionable property of expanding and contracting during their application and must be used in semi-melted condition in the patient's mouth.

The composition of material of our invention possesses all of the above-mentioned, and other, desirable chemical and physical attributes and none of the objectionable properties described, and presents dental impression materials posse...

ing valuable attributes of the highest practical value.

It is desirable that a dental impression material should contain a liquid of some kind in order to produce a composition of plastic properties for allowing the production of impressions and that the liquid should be readily and rapidly evaporable in order that its retention in the mouth may require a minimum of time in order not to unduly inconvenience the patient.

It is evident that the moisture content should be as nearly uniform as possible throughout the mass during and after the formation of the impression in order that the impression may be obtained and retained without undue distortion, and that a rapidly evaporable liquid is much more effective in this respect than is one of slow evaporable properties.

A further necessary property of such a liquid is that it should be a solvent for those elements of the composition which act as binders for the insoluble elements, in order that the binding properties are uniform throughout the mass, thus forming a uniform composition of matter during its application for the production of impressions and thereafter for further operations.

The most important properties of a solvent adaptable for dental impression materials are that it must be non-poisonous, non-toxic, and as non-irritating as possible. It must be non-poisonous and non-toxic because it is introduced into the mouth of the patient and must remain therein for a period of time, during which it should not be absorbed by the tissues of the mouth with resulting injurious effects, and it must be as non-irritating as possible as the mass must remain in undisturbed position during the impression period. Any irritating effect is liable to cause the patient to contract, expand, or otherwise change the position of the mouth contour, thus disturbing and destroying the proper formation of the impression mass.

It is evident that compositions of matter adapted for dental impression materials must contain some compound or compounds, or fillers, which are capable of setting into a mass of sufficient hardness as to allow of the necessary operations upon the composition after the dental impressions have been made, and that these fillers must be chemically and physically compatible with the other ingredients.

These fillers must be of such composition that they will form a uniform, pliable, workable mass when inserted within the mouth for the making of impressions; they must not adhere to the mouth tissues; they must not unduly impede the evaporation of the solvent; they must not crumble, crack, or flake while in the mouth or while in molding form; and they must be non-poisonous, non-toxic, and non-irritating.

It is evident, therefore, that considerable care and research are necessary in order to determine and formulate a proper composition of matter adapted for the production of dental impressions.

We have found that ethyl alcohol is particularly adapted for solvents in compositions of the described character, as it is non-poisonous, non-toxic, and practically non-irritating. It produces a mild anaesthesia, dehydrates the surface of the mucous membranes, and prevents gagging.

Other solvents have been suggested for this purpose but they are not free from the objectionable properties previously mentioned. Methyl alcohol is poisonous, toxic, and much more irri-

tating that ethyl alcohol. Aromatic oils are extremely irritating and have a deleterious effect upon the mouth tissues.

It is evident from the foregoing description of the requirements necessary in a proper dental impression material that considerable research was necessary in order to determine the other ingredients which will co-act with ethyl alcohol to produce the desired effect.

We have found that a composition of matter having the described valuable and necessary properties can be obtained by a composition of matter formed from ethyl alcohol, castor oil, blown castor oil, or other oxidized, polymerized, sulphonated, esterified, hydrogenated, or acetylated products of castor oil, certain gums, an accelerator (or thickener) for such gums, and a filler.

The ethyl alcohol soluble gums we have found suitable for our purpose are Manila gum, Pontianak gum, and Philippine gum.

Among the accelerators (or thickeners) included in our invention are calcium chloride, zinc chloride, magnesium chloride, calcium nitrate, zinc nitrate, magnesium nitrate, calcium aluminate, calcium oxide, zinc oxide, and magnesium oxide, but we do not limit ourselves to these specific accelerators.

Among the mineral, vegetable, and animal fillers suitable for use in our composition of matter are talc, China clay, asbestos, mica, ochre, iron oxide, silica, infusorial earth, diatomaceous earth, graphite, magnesium silicate, aluminum silicate, calcium carbonate, wood flour, cotton linters, ground cork, ground wool, and silk fibre, but we do not limit ourselves to these specifically mentioned fillers.

We give the following formulae as examples of compositions of matter according to our invention, but we do not limit ourselves to these specifically mentioned chemicals or proportions as it is evident that they may be varied without going beyond the scope of our invention as described and claimed:

#### FORMULA 1

|                    | Parts |
|--------------------|-------|
| Manila gum         | 40    |
| Ethyl alcohol      | 33    |
| Magnesium silicate | 95    |
| Raw castor oil     | 16    |
| <b>B</b>           |       |
| Zinc oxide         | 9     |
| Raw linseed oil    | 5     |

#### FORMULA 2

|                  | A  |
|------------------|----|
| Manila gum       | 36 |
| Ethyl alcohol    | 32 |
| China clay       | 85 |
| Blown castor oil | 20 |

|                 | B  |
|-----------------|----|
| Magnesium oxide | 10 |
| Raw castor oil  | 4  |

#### FORMULA 3

|                       | A  |
|-----------------------|----|
| Philippine gum        | 40 |
| Ethyl alcohol         | 32 |
| Calcium carbonate     | 80 |
| Acetylated castor oil | 15 |

|                   | Parts |
|-------------------|-------|
| <b>B</b>          |       |
| Calcium oxide     | 4     |
| Calcium aluminate | 4     |
| Raw linseed oil   | 5     |

**FORMULA 4**

|                    | Parts |
|--------------------|-------|
| <b>A</b>           |       |
| Philippine gum     | 39    |
| Ethyl alcohol      | 30    |
| Magnesium silicate | 93    |
| Raw castor oil     | 14    |

**B**

|                |   |
|----------------|---|
| Zinc oxide     | 8 |
| Raw castor oil | 4 |

**FORMULA 5**

|                  | Parts |
|------------------|-------|
| <b>A</b>         |       |
| Pontianak gum    | 38    |
| Ethyl alcohol    | 32    |
| China clay       | 86    |
| Blown castor oil | 18    |

**B**

|                 |    |
|-----------------|----|
| Magnesium oxide | 10 |
| Raw linseed oil | 5  |

**FORMULA 6****A**

|                       |    |
|-----------------------|----|
| Pontianak gum         | 40 |
| Ethyl alcohol         | 33 |
| Calcium carbonate     | 82 |
| Acetylated castor oil | 14 |

**B**

|                   |   |
|-------------------|---|
| Calcium oxide     | 4 |
| Calcium aluminate | 4 |
| Raw castor oil    | 4 |

All of the above-mentioned parts refer to relative weights of the various materials.

While it is not absolutely necessary to mix the accelerator with an oil before adding it to the mixtures "A," we prefer to do so as it allows of a more complete and uniform incorporation of it into mixtures "A."

While the mentioned oils are suitable for our purposes, we prefer to employ blown castor oil as it produces a more readily applicable material than the others.

In the application of our materials for making dental impressions, we prefer to retain mixtures "A" and "B" separate from each other and to mix them together with thorough stirring for one or two minutes before applying them.

The above-described dental impression materials of our invention are non-poisonous, non-toxic, practically non-irritating, and tasteless; they will not crack, crumble, or flake during the operations to which they are submitted; they are readily workable in the mouth, producing clean, clear, and exact impressions at comfortable temperatures to the patient; they set rapidly in the mouth, from which they are easily and readily removed; they do not gag the patient; they are easily removed from the mold; and they possess the further valuable property that they do not contract or expand during the performance of all necessary operations, thus insuring that the casts produced therefrom coincide in every particular with the original mouth impressions.

While we have described our compositions of

matter as specifically applicable for the formation of dental impressions, we do not limit ourselves to their application for this particular purpose, as their composition and physical and chemical properties makes them useful and valuable for all purposes where their properties are such as to successfully meet such required conditions.

Where we employ the word "oil," the word "accelerator," the word "gum," and the word "filler" in our claims, we include both a single member of each said group and a mixture of a plurality of members of each said group.

We do not limit ourselves to the chemicals and quantities thereof as specifically set forth in our specification as these are given solely for the purpose of clearly describing our invention, and they may be varied without going beyond the scope of our invention.

## 20. What we claim is:

1. A composition of matter adapted for the production of dental impressions comprising ethyl alcohol, at least one member selected from the group consisting of castor oil, blown castor oil, polymerized castor oil, oxidized castor oil, sulphonated castor oil, esterified castor oil, hydrogenated castor oil and acetylated castor oil; an ethyl alcohol soluble gum, at least one accelerator for said gum and at least one filler.

30. 2. A composition of matter adapted for the production of dental impressions comprising ethyl alcohol, blown castor oil, at least one ethyl alcohol soluble gum, at least one accelerator for said gum and at least one filler.

35. 3. A composition of matter adapted for the production of dental impressions comprising ethyl alcohol, blown castor oil, Manila gum, at least one accelerator for said gum and at least one filler.

40. 4. A composition of matter adapted for the production of dental impressions comprising ethyl alcohol, blown castor oil, Manila gum, magnesium oxide and at least one filler.

5. A composition of matter adapted for the production of dental impressions comprising ethyl alcohol, blown castor oil, Manila gum, magnesium oxide and magnesium silicate.

6. A composition of matter adapted for the production of dental impressions comprising ethyl alcohol, blown castor oil, Manila gum, magnesium oxide, magnesium silicate and asbestos fibre.

7. A composition of matter adapted for the production of dental impressions comprising ethyl alcohol, castor oil, at least one ethyl alcohol soluble gum, at least one accelerator for said gum and at least one filler.

8. A composition of matter adapted for the production of dental impressions comprising ethyl alcohol, castor oil, Philippine gum, and at least one accelerator for said gum and at least one filler.

9. A composition of matter adapted for the production of dental impressions comprising ethyl alcohol, castor oil, Philippine gum, zinc oxide and at least one filler.

10. A composition of matter adapted for the production of dental impressions comprising ethyl alcohol, castor oil, Philippine gum, zinc oxide and China clay.

11. A composition of matter adapted for the production of dental impressions comprising ethyl alcohol, castor oil, Philippine gum, zinc oxide, China clay and silk fibre.

12. A composition of matter adapted for the

production of dental impressions comprising ethyl alcohol, polymerized castor oil, at least one ethyl alcohol soluble gum, at least one accelerator for said gum and at least one filler.

13. A composition of matter adapted for the production of dental impressions comprising ethyl alcohol, polymerized castor oil, Pontianak gum, at least one accelerator for said gum and at least one filler.

14. A composition of matter adapted for the production of dental impressions comprising ethyl alcohol, polymerized castor oil, Pontianak gum, calcium oxide and at least one filler.

15. A composition of matter adapted for the production of dental impressions comprising ethyl alcohol, polymerized castor oil, Pontianak gum, calcium oxide and silica.

16. A composition of matter adapted for the production of dental impressions comprising ethyl alcohol, polymerized castor oil, Pontianak gum, calcium oxide, silica and cotton linters.

CONSTANT A. BENOIT.  
HERMAN C. FUCHS.